

# United States Patent Office

3,433,640

Patented Mar. 18, 1969

1

3,433,640

## PHOTOGRAPHIC SILVER HALIDE LIGHT-SENSITIVE MATERIAL

Fumihiro Nishio, Yoshiyuki Nakazawa, and Kintaro Nasu, Kanagawa, Japan, assignors to Fujishashin Film Kabushiki Kaisha, Kanagawa, Japan  
No Drawing. Filed Nov. 8, 1965, Ser. No. 506,842  
Claims priority, application Japan, Nov. 13, 1964,  
39/63,973

U.S. Cl. 96—107  
Int. Cl. G03c 1/28

10 Claims

This invention relates to photographic silver halide sensitive materials and to silver halide emulsions for photographic materials.

Photographic silver halide emulsions are generally produced by dispersing crystals of silver halide such as silver iodide, bromide and chloride in gelatin, polyvinyl alcohol or other high molecular electrolytes as a protective colloid and are applied as a light-sensitive material on a support of paper, glass, nitrocellulose, acetylcellulose, polyamide, polyester, polycarbonate and other synthetic high molecular materials in a thin film whereby photographic films, plates and papers are obtained.

We have found that the photographic characteristics can be remarkably improved by adding thiazoline-2-thiones to such light sensitive material during production or with the starting materials.

That is to say, the present invention is characterized by incorporating in a light sensitive material during production or with the starting materials thereof at least one of the thiazoline-2-thiones represented by the following general formula:



in which R<sub>1</sub> represents lower alkyl-, cycloalkyl-, aryl- or pyrimidyl- methyl group, R<sub>2</sub> represents alkylene group, R' and R'' represent hydrogen, lower alkyl-, hydroxy-alkyl- or aryl group, and R' and R'' may be linked to each other.

Illustrative of the compounds used in this invention are:

Compound 1.



2

Compound 2.



Compound 3.



Compound 4.



Compound 5.



Compound 6.



Compound 7.



55 The compound may be added in a silver halide emulsion at any step, but it is preferable to add the above compound, as the crystal or as a solution, when the crystals of silver halide are formed or ripened after washing with water, or just before the photographic silver halide emulsion is dissolved and coated on a support. The compound may be incorporated in, for example, an adjacent layer of the photographic silver halide emulsion layer (therefore, the term "silver halide emulsion layer" in the specification and claims includes the layers adjacent to the emulsion layer). More particularly, if the compound contained in gelatin or other protective colloid is added during production, the dispersion thereof can be favorably effected. Moreover, a light sensitive material may be treated with a solution containing the compound.

60 65 70 The first object accomplished by our invention is to make a blue-black tone of developed silver image of a

light sensitive material, in particular, photographic paper or positive photographic material and the second object is to raise the sensitivity of a light sensitive material.

Example 1

20 ml. of 0.3% methanol solution of the Compound 1 was added to 1 kg. of an adherent photographic paper emulsion containing 21.5 g. of silver chloride, to which 20 ml. of 6% aqueous solution of formalin was further added, and coated on baryta paper. The thus obtained photographic paper was exposed and developed at 20° C. for 1 minute by the use of the following developer after diluting to 1:1.

|                                 | G.  |
|---------------------------------|-----|
| N-methyl-p-aminophenol sulphate | 2   |
| Anhydrous sodium sulfite        | 30  |
| Hydroquinone                    | 7   |
| Sodium carbonate (monohydrate)  | 53  |
| Potassium bromide               | 1.5 |
| Water to 1000 ml.               |     |

After the developing treatment, it was dipped in a stop bath of 1.5% acetic acid solution for 15-20 seconds, fixed for 10 minutes in an acidic hardening fixing solution and washed with water for 60 minutes in water flow. Thereafter, the developed material was then subjected to the 25 hot-glaze or natural drying.

In carrying out this invention, images having a satisfactory blue-black tone could be obtained, while images having a brownish-black tone were obtained in the case of no addition of the compound (development, stopping 30 fixing, water washing and drying were similar to in the former).

Example 2

30 ml. of 0.3% methanol solution of the Compound 2 was added to 1 kg. of an enlargement photographic paper emulsion containing 25 g. of silver chlorobromide (silver bromide 30 mol percent), coated on a support similarly to Example 1 and dried. The resulting photographic paper, being exposed similarly to Example 1, was developed for 2 minutes at 20° C., fixed and washed with water. In this photographic paper to which the Compound 2 had been added, the initial developing velocity was rapid, the sensitivity was increased by 10% and images having a blue-black tone were obtained, as compared with images having a brownish-black tone in another photographic paper to which it had not been added.

Example 3

30 ml. of 0.3% methanol solution of the Compound 2 and 15 ml. of 0.1% aqueous solution of 1-phenyl-5-mercaptotetrazole as a fog inhibitor were added to 1 kg. of an adherent photographic paper emulsion containing 23 g. of silver chlorobromide (silver bromide 7 mol percent), coated on a support similarly to Example 1 and dried. The resulting photographic paper, being exposed as in Example 1, was developed at 20° C. for 1 minute 30 seconds, fixed, washed with water and dried. In this photographic paper, no fog increase was observed and an image having a blue-black tone was obtained without delaying the initial development, as compared with an image having a neutral black tone in the case of no addition of the compound.

Example 4

When the procedure as in Example 1 was repeated using 60 ml. of a 0.3% methanol solution of Compound 4 instead of Compound 1, almost same brown-black images as in Example 1 were obtained.

Example 5

40 ml. of 0.2% methanol solution of the Compound 6 was added to 1 kg. of a micro-positive emulsion containing 35 g. of silver chlorobromide (silver bromide 45 mol percent), coated on a triacetylcellulose film support to which a subbing layer had been previously applied, and

dried. The film thus resulting, being exposed similarly to Example 1, was developed at 20° C. for 2 minutes, fixed, washed with water and dried. This film gave a good image of neutral black tone, as compared with an image of brownish-black tone obtained in the case of no addition 5 of the compound.

Example 6

To 1 kg. of a fine grain positive emulsion containing 50 g. of silver iodobromide (silver iodide 1.5 mol percent) was added the compound of our invention as shown 10 in Table I. The composition was coated on a triacetylcellulose film support having a subbing layer, followed by drying. The thus obtained film, after exposure, was developed at 20° C. for 5 minutes by the use of the following developer and then was fixed, washed with water 15 and dried.

|                                 | G.   |
|---------------------------------|------|
| N-methyl-p-aminophenol sulphate | 0.3  |
| Anhydrous sodium sulfite        | 38.0 |
| Hydroquinone                    | 6.0  |
| Sodium carbonate (monohydrate)  | 22.5 |
| Citric acid                     | 0.7  |
| Potassium bromide               | 0.9  |
| Potassium metabisulfite         | 1.4  |
| Water to 1000 ml.               |      |

TABLE I

| Compound | Amount added       | Specific sensitivity | Gamma | Fog  |
|----------|--------------------|----------------------|-------|------|
| 2-----   | 0                  | 100                  | 3.1   | 0.05 |
|          | 6×10 <sup>-3</sup> | 107                  | 3.1   | 0.05 |
|          | 2×10 <sup>-2</sup> | 129                  | 3.3   | 0.05 |
|          | 6×10 <sup>-2</sup> | 162                  | 3.5   | 0.05 |
|          | 2×10 <sup>-1</sup> | 200                  | 3.5   | 0.06 |
|          | 6×10 <sup>-3</sup> | 110                  | 3.1   | 0.05 |
| 3-----   | 2×10 <sup>-3</sup> | 135                  | 3.3   | 0.05 |
|          | 6×10 <sup>-2</sup> | 170                  | 3.3   | 0.06 |
|          | 2×10 <sup>-1</sup> | 230                  | 3.5   | 0.07 |
|          | 6×10 <sup>-3</sup> | 105                  | 3.1   | 0.05 |
|          | 2×10 <sup>-2</sup> | 125                  | 3.1   | 0.05 |
|          | 6×10 <sup>-2</sup> | 150                  | 3.1   | 0.05 |
| 5-----   | 2×10 <sup>-1</sup> | 180                  | 3.3   | 0.05 |

In the case of thus carrying out our invention, the sensitivity alone could be raised, by increasing the amount of the compound, without substantially affecting the gamma and fog.

Example 7

To 100 g. of a photographic emulsion containing 2.8 g. of silver chloride was added a M/100 methanol-acetone (4:1) solution of the Compound 1, 2 or 7 in an amount as shown in Table II, coated on a glass plate to be 6 ml. emulsion/200 cm.<sup>2</sup> and dried.

The resulting photographic plate, after exposure to 50 light, was developed at 20° C. for 3 minutes by the developer having the following composition and was then fixed, washed with water and dried.

|                                 | G. |
|---------------------------------|----|
| N-methyl-p-aminophenol sulphate | 3  |
| Anhydrous sodium sulfite        | 45 |
| Hydroquinone                    | 12 |
| Sodium carbonate (monohydrate)  | 80 |
| Potassium bromide               | 2  |
| Water to 1000 ml.               |    |

TABLE II

| Compound | Amount added (ml.) | Specific Sensitivity | Tone of Image      |
|----------|--------------------|----------------------|--------------------|
| 1-----   | 0                  | 100                  | Brownish black.    |
|          | 2                  | 162                  | Weak blue black.   |
|          | 4                  | 182                  | Strong blue.       |
|          | 8                  | 245                  | Do.                |
| 2-----   | 2                  | 151                  | Weak blue black.   |
|          | 4                  | 170                  | Strong blue black. |
|          | 8                  | 229                  | Do.                |
|          | 2                  | 162                  | Do.                |
| 7-----   | 4                  | 257                  | Do.                |
|          | 8                  | 269                  | Do.                |

What is claimed is:

1. A photographic silver halide sensitive material comprising a support and a silver halide emulsion layer, said layer containing at least one compound selected from

5

the group consisting of compounds represented by the general formula:



5

and, a compound represented by the general formula:



10

5. A material as defined in claim 1 wherein said compound is



15

6. A material as defined in claim 1 wherein said compound is



20

7. A material as defined in claim 1 wherein said compound is



25

8. A material as defined in claim 1 wherein said compound is



30

9. A material as defined in claim 1 wherein said compound is



35

10. A material as defined in claim 1 wherein said compound is

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

6

5. A material as defined in claim 1 wherein said compound is



10

6. A material as defined in claim 1 wherein said compound is



15

7. A material as defined in claim 1 wherein said compound is



20

8. A material as defined in claim 1 wherein said compound is



25

9. A material as defined in claim 1 wherein said compound is



30

10. A material as defined in claim 1 wherein said compound is

#### References Cited

#### FOREIGN PATENTS

660,222 2/1965 France.

70 J. TRAVIS BROWN, Primary Examiner.

J. R. EVERETT, Assistant Examiner.

75 96-65, 109

U.S. Cl. X.R.